

# UNITED STATES PATENT OFFICE.

TRUMAN S. FULLER, OF SCHENECTADY, NEW YORK, ASSIGNOR TO GENERAL ELECTRIC COMPANY, A CORPORATION OF NEW YORK.

## ALLOY.

1,273,762.

Specification of Letters Patent. Patented July 23, 1918.

Application filed May 24, 1917. Serial No. 170,733.

To all whom it may concern:

Be it known that I, TRUMAN S. FULLER, a citizen of the United States, residing at Schenectady, county of Schenectady, State 5 of New York, have invented certain new and useful Improvements in Alloys, of which the following is a specification.

My present invention comprises a new alloy containing aluminum, magnesium, zinc 10 and either iron, chromium, cobalt, nickel, titanium or manganese, or a mixture of the same.

The addition of iron or one of the above-described equivalents increases the tensile 15 strength, hardness and stiffness of alloys containing aluminum, magnesium and zinc. Preferably the metal of the iron group is present in amounts of about 1 to 3%.

When preparing an alloy embodying my 20 invention, containing iron for example, the aluminum is melted and the iron is added either as substantially pure iron, or as an alloy of aluminum and iron, until a homogeneous alloy containing the desired amount 25 of iron is produced by the solution of the iron in the aluminum. The desired proportion of zinc is then added to the melted alloy. Finally the magnesium is added and the alloy is immediately cooled as by casting 30 or in any suitable manner. Alloys containing chromium, cobalt, nickel, titanium or manganese may be made in a similar manner.

The alloy is worked into desired form by 35 forging, rolling or drawing. The first stage of mechanical working is carried out while the metal is at about 450° C., but after ductility has been imparted the metal may be worked at ordinary temperatures.

40 Preferably the alloys embodying my invention contain about 6 to 12% of zinc, about  $\frac{1}{2}$  to 2½% of magnesium, about 1 to 3% iron or equivalent metals, such as chromium, cobalt, nickel, titanium and manga-

nese, the balance totaling 100% consisting 45 of aluminum, although these proportions may be departed from when special properties for special uses are desired.

The following specific examples illustrate the improvement in tensile strength effected 50 by iron or equivalent metal. An alloy consisting of about 92.75% aluminum, 6% zinc, 1.25% magnesium has an ultimate tensile strength of about 46,100 pounds per sq. in. An alloy of 90.75% aluminum, 6% zinc, 55 1.25% magnesium and 2% iron has an ultimate tensile strength of 69,600 pounds. In other words, the substitution of 2% aluminum by 2% iron effects an increase in tensile strength of over 50%. An alloy of 60 86.75% aluminum, 12% zinc and 1.25% magnesium has an ultimate tensile strength of 53,600 pounds. By replacing 3% of the aluminum by 3% iron the ultimate tensile strength is increased to 63,000 pounds or 65 about 18%.

I desire by the appended claims to cover not only an alloy of aluminum, magnesium, zinc and iron but also metals equivalent to iron for this purpose, such as chromium, 70 cobalt, nickel, titanium or manganese.

What I claim as new and desire to secure by Letters Patent of the United States, is,—

1. An alloy containing aluminum, at least 75 several per cent. of zinc, at least about one-half per cent. of magnesium and at least about one per cent. of iron.

2. An alloy containing aluminum, at least 80 several per cent. of zinc, at least about one-half per cent. of magnesium and about one to three per cent. of iron.

3. An alloy consisting of about 6 to 12 per cent. of zinc, about  $\frac{1}{2}$  to 2½ per cent. of magnesium, about 1 to 3 per cent. of iron and the balance of aluminum. 85

In witness whereof, I have hereunto set my hand this 23rd day of May, 1917.

TRUMAN S. FULLER.